

# UNITED STATES PATENT OFFICE.

EUGENIO MARCHESE, OF GENOA, ITALY.

## PROCESS OF EXTRACTING COPPER FROM ITS ORES.

SPECIFICATION forming part of Letters Patent No. 326,760, dated September 22, 1885.

Application filed November 1<sup>st</sup>, 1884. (No specimens.) Patented in Germany September 13, 1884; in England September 23, 1884, No. 12,725, and in Italy October 13, 1884, XXXIV, 309.

*To all whom it may concern:*

Be it known that I, EUGENIO MARCHESE, a citizen of Italy, residing at Genoa, in the Kingdom of Italy, have invented a new and useful 5 Process of Extracting Copper from its Ores, of which the following is a specification.

The practical application of electrolysis to the metallurgy of copper has gone no further than the refining of impure metallic copper. 10 All the processes proposed for the practical electrolysis of ores or regulus have completely failed. The reason thereof is, above all, to be ascribed to the presence of a great percentage of iron in these materials, (ore or regulus,) 15 and the great difficulty, that never was surmounted, of obtaining pure and compact electrolytic copper from anodes or solutions, or both, containing iron in great quantity. Other economical and practical difficulties attended 20 the processes that have been proposed, and in effect no one of these processes has been brought into actual application, although a long time has elapsed since they were proposed. A number of these processes had been 25 proposed on the principle of the electrolysis of sulphate of copper brought beforehand into solution, the sulphate having to be obtained by an acid lixiviation of the proposed materials after they had been submitted to a 30 complete roasting. (Cobley's patent.) In this process the iron sulphate which accompanies the copper sulphate in the solution prepared by means of the roasted materials must be separated by a special chemical operation 35 from the copper sulphate before the solution containing this salt could be employed in the electrolytic vessels, (voltameters.) No hint is given how the anodes are to be prepared, and the difficulty attending a special 40 chemical separation of iron in the solution, the impossibility of obtaining a complete roasting of the ore or regulus, and so avoiding the loss of a portion of the copper they contain, along with the great amount of mechanical power required for the dissociation 45 of sulphate of copper when a soluble anode is not provided for, render that process inapplicable in practice. Mr. Elhington, (Elhington's patent,) who proposed and carried on 50 successfully the refining of impure copper by electrolysis, suggests in his specifications to

apply the same process to ores or regulus taken from any stages of the usual metallurgical process, although he declares to prefer blister or pimpled copper—that is, impure metallic copper. In fact, the practical extraction of pure copper from ore or regulus by submitting it to the same process as that of refining copper, as Mr. Elhington suggests, has never been carried on effectually, because it is not practicable. The iron contained in the ore or regulus, which can amount even to forty or forty-five per cent., renders the process as suggested by Elhington absolutely impracticable; and it is a well-known fact that even in the 65 electrolytic refining of impure copper which contains but a very small percentage of iron the copper-sulphate solution in the electrolytic vessels must be changed as soon as a sensible quantity of the iron has been converted by electrolytic oxidation into iron sulphate, and new copper-sulphate solution, free from iron sulphate, must be supplied to the electrolytic vessels. The reason thereof is the formation at the anode of the ferric salts, 70 and the reduction of the ferric salts into ferrous salts at the cathode. Such a transformation, which requires a less electro-motive force, goes on in a proportion so much the greater, the greater is the quantity of the iron sulphate in the solution, and along with that phenomenon the useful electrolysis of copper subsides proportionally. On the other hand, the copper deposit wants the compactness and purity that are required for practical 75 purposes.

The process that forms the subject of my present invention obviates all the above-stated difficulties, and its most important result is to obtain pure and compact electrolytic copper 90 from anodes made of regulus containing iron in whatever quantity and employing copper-sulphate solutions containing whatever quantity of sulphate of iron. All ores or regulus or other copper material whatever can also be 95 practically treated by my process. The presence of iron in the anode, which I make of regulus, not only does not hinder the efficiency of the process, but is converted into a powerful economical auxiliary, as the economical feature of my process is the utilization 100 of the iron contained in the anode for

electrolytic dissociation of the sulphate of copper contained in the solution extracted from the roasted ores or regulus. It is well known that the sulphate of copper requires for dissociation an electro-motive force of 1.2 volt 5 in my process by the oxidation of the iron sulphide of the anodes which takes place by the electric current, a large portion of that electro-motive force is gratuitously supplied, 10 and the electrolysis goes on, practically requiring no more than 0.4 to 0.5 volt for the chemical dissociation and deposition of copper on the cathode. As for the corresponding difficulty arising in the proposed processes 15 from the presence of large quantities of sulphate of iron in the solution, this is completely obviated in my process by means of a continually-active circulation of the solution from the electrolytic vessels to the tanks in which 20 the roasted material is submitted to lixiviation.

My process for extracting chemically-pure copper by electrolysis from copper ores, copper regulus, or other copper materials is practically carried on thus: The copper ore or 25 copper regulus, or other copper material from which the copper has to be extracted, whatever be the proportion of iron it happens to contain, is roasted in kilns or other suitable 30 furnaces, as is done in usual metallurgical processes. (Mansfeld, Freiberg, &c.) The object of this roasting being the conversion of the sulphides into oxides and the conversion of sulphur into sulphuric acid by the ordinary 35 means of the lead chambers, (unless sulphuric acid is otherwise available at less cost,) such roasting of the ore or regulus does not require to be a complete one, as the portion that has not been converted into oxides will serve for 40 the formation of the anodes after it has been separated from the roasted portion that has become soluble in sulphuric acid and been extracted by lixiviation, as sulphate of copper, (and sulphate of iron.) If that residual part 45 of the lixiviation be not sufficient to afford the quantity of anodes required by the process, a convenient portion of the ore or regulus is added accordingly. The economy of the 50 process consisting in availing oneself of the iron contained in the anodes for the electrolysis of the copper contained in the solution, there must be a consequent relation between the quantity of iron contained in the anodes and the quantity of copper that ought to be 55 brought in the process in the state of sulphate in solution, and to determine that proportion I avail myself of the fact that two chemical equivalents of iron dissociate in my process three equivalents of the copper sulphate contained in the solution. Thus, if I have 60 regulus containing, say, thirty-five per cent. of copper and forty per cent. of iron, one hundred parts of that regulus cast into anode-plates 65 will dissociate approximately  $40 \times \frac{3 \times 32}{2 \times 28}$  parts of copper sulphate of the solution, assuming that 32 and 28 are approximately the chemi-

cal equivalents of copper and iron. In this case nearly one-third of the regulus that I have to treat must be reduced in form of anodes, 70 and the other two-thirds into solution. An analogous calculation can be made in every case; also, in order to make the anodes for the process, I take the residue of the ore or regulus, whether alone or with addition of a portion of ore or regulus; or I may use only the ore or regulus, if the residue of the roasted material should be inconvenient for that purpose. The way I make these anodes is by smelting the materials above mentioned (residue of roasting, or ores, or regulus, or a mixture of them), in a cupola-furnace or other furnace, casting the smelted metallic product (copper, iron, and sulphur, composing the copper regulus) into cast-iron molds having the 85 dimensions suitable for my plant—say, two feet six inches wide, two feet six inches deep, and one and three-sixteenths inch to one and nine-sixteenths inch thick. In the cast-iron mold, which is set vertically on the ground, a small 90 band or wire of copper is held in suspension during the casting of the smelted regulus, which after the cooling of the plate remains inserted in it, and affords an easy means for connecting the anode to the general copper 95 conductors of the electric current when it is placed into the electrolytic vessel or voltameter. If in the casting of the anodes, as above described, there are any defects, they are broken up and passed into the roasting operation with the ores or regulus intended for the 100 formation of solution and sulphuric acid, as was hereinbefore said, so that nothing of the material is lost or has to be put aside. The anodes so obtained I place in suitable vessels 105 or voltameters, each of them containing, say, fifteen or twenty anodes. The anodes, placed vertically, repose on two longitudinal pieces of wood placed on the bottom of the voltameter, so that between the under side of the anodes and the bottom of the voltameter a certain space (say, six inches high) remains free. To hold the anodes in their upright position and at a fixed distance, I place two wooden 110 racks in the voltameter, between whose teeth 115 the sides of the anodes are confined. The connection of the anodes with the copper conductors of the current is then made by the copper band or wire inserted in them. Between the anodes are placed the cathodes of electrolytic copper in communication with the conductors of the other pole, as is well known. The distance between anodes and cathodes I 120 make about two inches. The solution that is to operate in these vessels or voltameters so 125 provided with their anodes and cathodes I provide, as above said, from the roasted material (ore or regulus) by means of acid solution and lixiviation. The required sulphuric acid is produced in the lead chambers from 130 the sulphur contained in the roasted materials in the usual way, and I take the first chamber sulphuric acid. As the ore or regulus contains more sulphur than is necessary to

5 sulphatize the iron of the anodes, and as by roasting a large portion of the oxidized iron becomes insoluble, I obtain more sulphuric acid than is necessary for the requirements of the process. The surplus is sold.

10 The solution and lixiviation of the roasted materials I effect in the known ways, avail-  
ing myself of the knowledge of the quantity  
of the copper that I dissociate from the solu-  
tion by sulphatization of the iron contained  
in the anode, to regulate proportionately the  
addition of sulphuric acid in the lixiviating-  
tanks, so as to maintain the solution but  
slightly acid. It is by no means required in  
15 my process that the lixiviation be complete  
and absolute. The residue I pass to the smelt-  
ing of the anodes; and to avoid the possibility  
of loss of copper oxide I have only to add in  
the smelting some copper pyrites or iron py-  
rites. It is not required for the success of my  
20 process that the solution be saturated with  
copper sulphate. In fact, if it contains from one  
to two per cent. of copper, the proportion is  
quite sufficient. As to iron sulphate, the so-  
25 lution may, without inconvenience, contain  
any quantity. In fact, during the process the  
solution will be always charged with sulphate  
of iron so far as no physical inconvenience  
(crystallization of the salt) arises for its cir-  
30 culation.

35 The main features of my process, in what  
concerns the solution, is that the solution must  
continually circulate from the electrolytic ves-  
sels or voltameters, where the electric disso-  
ciation takes place, to the lixiviation tanks,  
40 where the roasted materials are submitted to  
the acid action in order to sulphatize and so  
to dissolve the oxides of copper and iron.  
This circulation can be arranged in different  
ways and by known means. The sole essen-  
45 tial point is that it shall take place continually  
in each electrolytic vessel or voltameter, and  
that the so circulating solution, after having  
passed through one, or a number of the vol-  
50 tameters, be carried to the lixiviation tanks,  
to be passed back from there to the voltame-  
ters, and so on continually. When the elec-  
tric current passes into the voltameter so dis-  
posed, and does its work of electrolysis, the  
55 copper of the anode is dissociated from sul-  
phur and deposits in the cathode. At the same  
time the iron of the anode is dissociated equally  
from sulphur and converted into sulphates,  
the electro-motive force arising from that  
60 chemical combination being employed in the  
dissociation of the sulphate of copper con-  
tained in the solution, with deposit also of  
copper on the cathode. Consequently the so-  
lution is gradually impoverished in sulphate of  
65 copper, and one of the objects of the circula-  
tion is to bring the impoverished solution into  
the lixiviation tanks in order that it can ap-  
propriate copper sulphate again and regain  
its original percentage of copper. This fact  
gives the practical means of arranging the  
mode of circulation. If the normal solution  
held, say, three per cent. copper, it can flow

through a number of voltameters until it is  
reduced to, say, one and a half per cent. be-  
fore being carried back to the lixiviating-  
tanks. Another object of the continuous cir-  
culation is that of maintaining the ferric salts  
and the ferrous salts in such a state of admix-  
ture in the solution passing through the vol-  
tameters as to hinder the dissociation of fer-  
rous salts which could take place, and the  
consequence of which (the solution being  
slightly acid) would be a development of hy-  
drogen at the cathode, and the consequent  
deposition of copper not in a solid and com-  
pact state, as in galvano-plastic, but dis-  
integrate and pulverulent, so as to fall down  
on the bottom of the voltameter. On the  
other hand, the immobility of the solution  
would give rise to the fact that the electric  
current would become specially absorbed by  
the reduction of the ferric salts, into ferrous  
ones instead of being employed exclusively in  
effecting the dissociation of the sulphides of the  
anodes and of the sulphates of the solution,  
with the consequent useful deposition of good  
electrolytic copper on the cathode. A good  
circulation to that effect I have obtained  
when about one-fifth of the solution contained  
in the voltameter passes through it by circu-  
lation during one hour. The copper I leave  
to accumulate on the cathode till it reaches  
sufficient thickness, as usual in the electrolytic  
refining of impure copper. The residues of  
the anodes, in which the sulphur that was first  
combined with copper and iron remains in  
the metalloid state, (so that it can burn like  
sulphur,) when they are so impoverished in  
metals that they are no longer effectual for the  
proper passing of the electric current, are  
taken away and passed into the roasting op-  
eration with the raw materials, (ore or regu-  
lus.) Thus nothing is lost of the copper they  
might still contain, and the metalloid sulphur  
contained affords an excellent material for  
sulphuric acid in the roasting operation. Nat-  
urally, if the materials (ore or regulus) contain  
even very small quantities of precious metals,  
those metals accumulate gradually in such re-  
sidual parts, which become continually richer  
until they can pass conveniently to a desilver-  
ing process. As the solution, circulating as  
above stated, takes continually a certain quan-  
tity of iron from the anodes, (and from the  
roasted material,) a portion of the same solu-  
tion, calculated on the daily increase of the  
iron sulphate so formed, must be daily brought  
out of the process. This portion is deprived  
of the copper contained by the known pro-  
cesses, or by a special electrolysis, where the  
copper falls on the bottom of the voltameter.  
The sulphate of iron can be crystallized if  
there be a convenient sale for it. Otherwise  
it is thrown away. As to the electrical ar-  
rangement, it can be carried on in different  
known ways. Owing to the practical diffi-  
culty of possessing good dynamos having a  
very small electro-motive force, I dispose a se-  
ries of voltameters in tension, so that for every

voltameter an electro-motive force of about one volt be available between the anodes and the cathodes. An electro-motive force of about 0.5 volt is necessary for the chemical dissociation, and the more that is given depends upon the plant employed. With large surfaces a saving in electro-motive power, and consequently in mechanical power, can be effected; but the electro-motive force must never go below the chemical reaction, which can be measured in every case. Above that required for such reaction the augmentation of the electro-motive force corresponds to a restriction of the surfaces—that is, of the plant of the process. However, too high an electro-motive force, besides being uneconomical, has very great inconveniences, as it can give rise to higher chemical reactions, which could produce polarization with very bad consequences. In all cases in copper electro-metallurgy the electro-motive force of one volt between anodes and cathodes should be considered as a maximum not to be surpassed.

Having thus described the nature of my in-

vention and the best means I know of carrying it into effect, I claim—

The herein-described process for the electrolytical extraction of copper from ores or regulus containing iron, which consists in smelting a portion of the ore or regulus and casting it into plates and roasting and lixiviating the other portion, and subjecting the plates to the action of the solution of sulphate of iron and sulphate of copper and an electric current, as described, the solution being made to circulate continuously between the electrolytic vessel and the solution-tank containing roasted ore for the purpose of maintaining sufficient sulphate of copper in the electrolysis, substantially as set forth.

In testimony whereof I have signed my name to this specification, in the presence of two subscribing witnesses, this 13th day of October, 1884.

EUGENIO MARCHESE.

Witnesses:

ROBERTO CATTANEO,  
TOMASO GREGORY.